

## [54] AGENTS FOR INHIBITING THE CORROSION OF IRON IN ACID SOLUTION

[75] Inventors: Lorenz Heiss, Hofheim, Taunus; Martin Hille, Bad Soden, Taunus, both of Germany

[73] Assignee: Farbwerte Hoechst Aktiengesellschaft vormals Meister Lucius &amp; Bruning, Frankfurt, Germany

[22] Filed: Dec. 21, 1971

[21] Appl. No.: 210,558

## [30] Foreign Application Priority Data

Dec. 28, 1970 Germany ..... P 20 63 987.6

[52] U.S. Cl. .... 252/147, 252/148, 252/149, 252/151, 252/395

[51] Int. Cl. .... C11I 7/34, C23g 1/06

[58] Field of Search ..... 252/149, 151, 147, 252/395, 87, 181; 260/607 B

## [56] References Cited

## UNITED STATES PATENTS

|           |         |                     |             |
|-----------|---------|---------------------|-------------|
| 2,078,256 | 4/1937  | Lieber et al. ....  | 252/77 X    |
| 2,121,823 | 6/1938  | Piggott ....        | 260/607 B X |
| 2,941,949 | 6/1960  | Saukaitis.....      | 252/151     |
| 3,060,156 | 10/1962 | Rassweiler.....     | 260/79      |
| 3,216,979 | 11/1965 | Sexsmith et al..... | 260/79.3    |
| 3,668,137 | 6/1972  | Gardner.....        | 252/151 X   |

Primary Examiner—Leon D. Rosdol

Assistant Examiner—Harris A. Pitlick

Attorney—Arthur G. Connolly et al.

## [57] ABSTRACT

Corrosion inhibiting agents having the formula



in which R<sub>1</sub> stands for an alkyl radical having 4 to 18 carbon atoms and bound in the 6-, 4- or 2-position to the benzene nucleus, R<sub>2</sub> stands for hydrogen, an alkyl radical having up to 9 carbon atoms, or a radical of the formula



A stands for one of the anions Cl<sup>(-)</sup>, Br<sup>(-)</sup>, I<sup>(-)</sup>, CH<sub>3</sub>OSO<sub>3</sub><sup>(-)</sup> and 1/2 SO<sub>4</sub><sup>(-x-)</sup> in a quantity which is equivalent to the number of the positively charged sulfur atoms in the total molecule of the formula I, and X stands for a lower alkyl radical, the radical -C<sub>2</sub>H<sub>4</sub>OH or a radical of the formula



in which n means an integer of 1 to 30 and m stands for 0 or 1 and wherein, if n is at least 3, in this formula II an amount of up to one third the radicals which are enclosed by the bracket [] can be replaced by radicals of the formula



8 Claims, No Drawings

## AGENTS FOR INHIBITING THE CORROSION OF IRON IN ACID SOLUTION

In the industry, the inhibition of the corrosion of iron and iron alloys constitutes a serious problem. The inhibition of the corrosion is particularly difficult when acids are used simultaneously.

Attempts have already been made to obtain an inhibition or reduction of the corrosion of iron or iron alloys by application of organic or inorganic compounds. As such corrosion inhibitors, the most various compounds such as higher molecular amines, quaternary ammonium compounds, organic phosphonium compounds, sulfonic acids, fatty acids, thio-ureas, mercaptans, alkyl sulfides and alkyl sulfoxides as well as heterocyclic compounds with oxygen, sulfur or nitrogen as hetero-atoms have been proposed.

Corrosion inhibitors are used mainly in the surface cleaning of iron and iron alloys, where, in general, aqueous acids are employed for the removal of rust, scales and the like. The action of the acid is to be controlled in such a manner that the surface impurities are attacked and the material itself remains unaffected. To reach this goal, special inhibitors are used.

The present invention provides new corrosion inhibitors which permit a better protection of iron and iron alloys in acid solution. The invention furthermore relates to the use of these new inhibitors in the known industrial processes, for example in the surface cleaning of metals, wherein iron or iron alloys are subjected to the action of acid solutions.

Accordingly, the present invention provides agents which inhibit the corrosion of iron or iron alloys in acid solution and which essentially consist of, or contain as the active component, compounds of the formula I



in which X represents an alkyl group having 1 to 4 carbon atoms, the group  $-\text{C}_2\text{H}_4-\text{OH}$  or a group of the formula II



in which n represents numbers from 1 to 30 and m represents 0 or 1 and wherein, if n is at least 3, in this formula II an amount of up to one-third of the radicals which are enclosed by the bracket can be replaced by radicals of the formula



R<sub>1</sub> represents a straight chain or branched alkyl group having 4 to 18 carbon atoms bound in the 6-, 4- or 2-position to the benzene nucleus, R<sub>2</sub> represents hydro-

gen, a straight chain or branched alkyl group having 1 to 9 carbon atoms or a group of the formula



in which X has the meaning given above, A represents the anions  $\text{Cl}^{(-)}$ ,  $\text{Br}^{(-)}$ ,  $\text{I}^{(-)}$ ,  $\text{CH}_3\text{OSO}_3^{(-)}$ ,  $1/2\text{SO}_4^{(-2)}$  in a quantity which is equivalent to the number of the positively charged sulfur atoms in the total molecule of the formula I.

In addition, it is advantageous to add to the corrosion inhibitors of the invention small amounts of up to about 15 percent by weight, referred to the sulfonium salts of the formula I, of alkynols, preferably propargyl alcohol. The new corrosion inhibitors may be applied together with other known corrosion inhibitors, other auxiliary agents, for example surface-active agents.

The sulfonium salts of the formula I used according to the invention as corrosion inhibitors can be prepared by transforming a monoalkyl- or dialkyl-benzene by chloromethylation into the corresponding alkyl- or dialkyl-benzyl chloride and reacting the latter with an alkali mercaptide of thioethylene glycol to obtain the corresponding thio-ether:



From the thio-ether, there can be obtained in known manner by reaction with alkylating agents, for example dimethyl sulfate, alkyl halides or similar compounds, the sulfonium salt. The sulfonium salts of thio-diethylene glycol, polythio-diethylene glycol and polythio-diethylene-glycol formal can be obtained by direct reaction of these thio-ethers with the corresponding alkyl-benzylchlorides.

The polythio-diethylene-glycol of the formula



may be prepared, for example according to the method described in "Houben-Weyl, Methoden der organischen Chemie," volume 14/2 (1963), page 586. The polythio-diethylene-glycol ethers or the polythio-diethylene-glycol formals can then be reacted in known manner with alkyl-benzyl halides to yield the corresponding alkyl-benzyl-sulfonium salts. The reaction can be carried out by mixing the substances with stirring, if necessary in the presence of solvents, at room temperature or, if necessary, while heating. An addition of metal halides, such as zinc chloride, has an accelerating effect in the reaction.

As alkyl benzenes which may be used as starting materials for the preparation of the sulfonium salts of the formula I, there may be mentioned, for example hexylbenzene, octylbenzene, tetra-propylene-benzene, dodecylbenzene, 4-tert.-butyltoluene, n-nonylbenzene

or an industrial alkyl-benzene mixture having alkyl groups of 12 to 18 carbon atoms.

The chloromethylation of these alkyl-benzenes can be effected in a manner known per se, for example by reaction with methylchloromethyl ether and Friedel-Crafts catalysts, for example zinc chloride or concentrated sulfuric acid. Depending on the quantity used of methylchloro-methyl ether, there can be introduced one or two chloromethyl groups into the benzene ring, so that compounds such, for example, as p-dodecylbenzyl-chloride, 2-chloro-methyl-4-tert.butyltoluene, 2,4-bis-chloromethyl-dodecylbenzene etc. are obtained.

The sulfonium salts of the formula I are excellent corrosion inhibitors for iron and iron alloys in acid solutions. They can be used in all those cases where aqueous or aqueous acid solutions are allowed to act on iron or iron alloys, for example in metal pickling baths for surface cleaning of iron or in similar processes.

The sulfonium salts of the formula I used according to the invention are added to the acid metal treating baths in such a quantity that their concentration in the baths is at least 0.05 percent by weight; preferably, the concentration is adjusted to a range of from 0.1 to 1.0 percent by weight. Though an upper limit for the concentration of the corrosion inhibitors of the invention does not exist, a concentration of 2.0 percent by weight will in general not be exceeded for economical reasons, the more so since a higher concentration in most cases does not improve the protection against corrosion. In special cases, the indicated concentrations may be higher or lower than the indicated limits, if necessary.

The preparation of the sulfonium salts of the formula I of the present invention is illustrated in the following Examples:

I. Preparation of p-tetrapropylenebenzyl-S.oxethyl-S-methylsulfonium-methosulfate

300 g (1 mole) of tetrapropylene-benzyl chloride, obtained in known manner from tetrapropylene-benzene and methyl-chloromethyl ether and zinc chloride or concentrated sulfuric acid were combined, while stirring, with 78 g (1 mole) of  $\beta$ -hydroxyethyl-mercaptan and then with 40 g (1 mole) of sodium hydroxide, and the whole was then stirred for 5 hours at 50° - 60° C. 200 ml of water and 200 ml of benzene were added, while continuing stirring, and the benzene phase was separated. The benzene solution was washed several times with water, dried and the solvent was removed by distillation. Tetrapropylenebenzyl- $\beta$ -oxethyl sulfide in the form of a light yellow oil was obtained in a yield of 335 g (= 98 percent) having a content of organically bound sulfur of 9.3 percent (theory 9.36 percent) and a molecular weight of 338 (theory 342).

126 g (1 mole) of dimethyl sulfate were added dropwise, at 40° C, while stirring, to the tetrapropylenebenzyl- $\beta$ -oxethyl sulfide and the whole was stirred for 2 hours. The p-tetrapropylenebenzyl-S-oxethyl-S-methyl-S-sulfonium-methosulfate was obtained in the form of a viscous oil with a yield of 461 g and was found to be clearly soluble in water.

II. Preparation of poly-thiodiethyleneglycol-formal-dodecylbenzyl-sulfonium chloride

122 g (1 mole) of thiidiethyleneglycol and 30 g (1 mole) of para-formaldehyde in 500 ml of benzene were combined with 20 g of a  $H^+$ -ion exchanger resin and heated under reflux, while removing in about about 5 hours about 17 ml of water by azeotropic distillation.

15 The ion exchanger was filtered off and the solvent was removed. The poly-thiodiethyleneglycol-formal obtained in the form of a viscous oil with a yield of 131 g was found to have a molecular weight (measured osmotically in benzene) of 546 and a content of bound formaldehyde of 22.7 percent.

20 The poly-thiodiethyleneglycol-formal was combined with 300 g (1 mole) of p-n-dodecylbenzyl chloride, 500 ml of isopropanol and 50 g of zinc chloride, and the mixture was heated for 8 hours under reflux. Then, 500 ml of benzene were added, while stirring, and the whole was washed several times with saturated aqueous NaCl-solution to remove the zinc chloride. The solvent was removed by distillation in a rotary evaporator. The poly-thiodiethyleneglycol-formal-dodecylbenzyl-

25 sulfonium chloride was obtained in the form of a highly viscous oil with a yield of 421 g. The product contained 10.5 percent by weight of ionogenically bound chlorine.

30 The following Examples show the advantageous anti-corrosive action of the sulfonium salts of the invention. For testing the inhibiting effect, cleaned and weighed iron plates (soft steel RST 37-2-05), having a size of 75  $\times$  10  $\times$  0.75 mm each, were treated at 80° C in an aqueous solution containing 80 percent by weight of hydrochloric acid and (a) 0.05 percent by weight, b) 0.1 percent by weight or (c) 0.15 percent by weight of one of the following inhibitors. Subsequently, the loss in weight of the plates and thus the steel removal were established and indicated as a measure for the anticorrosive effected attained.

35 In the tests, the inhibitors of the invention were compared with anticorrosives which do not fall within the scope of the present invention and which are indicated in the Table hereinafter sub No. 13 to 16. The results of these comparative tests demonstrate the superior anticorrosive effect of the sulfonium salts according to the invention.

40

| Product                          | Concentration, steel removal (loss) in g./m. <sup>2</sup> |    |    |
|----------------------------------|-----------------------------------------------------------|----|----|
|                                  | a                                                         | b  | c  |
| 1.                               | 120                                                       | 80 | 65 |
| 2.                               | 98                                                        | 60 | 52 |
| 3. Equimolar mixture of 1 and 2. | 100                                                       | 66 | 54 |

| Product                                                                                                                                    | Concentration, steel removal<br>(loss) in g./m. <sup>2</sup> | a      b      c |     |   |
|--------------------------------------------------------------------------------------------------------------------------------------------|--------------------------------------------------------------|-----------------|-----|---|
|                                                                                                                                            |                                                              | a               | b   | c |
| 4.                                                        | 135                                                          | 95              | 78  |   |
| 5.                                                        | 105                                                          | 64              | 54  |   |
| 6.                                                        | 320                                                          | 220             | 180 |   |
| 7.                                                        | 95                                                           | 72              | 60  |   |
| 8.                                                        | 108                                                          | 85              | 60  |   |
| 9. Equimolar mixture of 7 and 8.                                                                                                           | 94                                                           | 70              | 58  |   |
| 10.                                                       | 102                                                          | 84              | 56  |   |
| A                                                                                                                                          |                                                              |                 |     |   |
| B                                                                                                                                          |                                                              |                 |     |   |
| R = industrial alkyl mixture with 8-12 carbon atoms (in the compound, the groups A and B are distributed statistically over the molecule). |                                                              |                 |     |   |
| 11.                                                      | 151                                                          | 108             | 92  |   |
| 12.                                                     | 185                                                          | 142             | 106 |   |
| 13.                                                     | 1,250                                                        | 990             | 810 |   |

| Product | Concentration, steel removal<br>(loss) in g./m. <sup>2</sup> |       |       |
|---------|--------------------------------------------------------------|-------|-------|
|         | a                                                            | b     | c     |
| 14.     | 2,100                                                        | 1,530 | 1,100 |
| 15.     | 3,200                                                        | 2,050 | 1,550 |
| 16.     | 1,970                                                        | 1,390 | 1,160 |

We claim:

1. An acid metal treating bath consisting essentially of hydrochloric acid and as a corrosion inhibitor 0.05 to 2.0 percent by weight of a compound of the general formula



in which X represents an alkyl group having 1 to 4 carbon atoms, the group  $-\text{C}_2\text{H}_4-\text{OH}$  or a group of the formula II



in which n represents numbers from 1 to 30 and m represents 0 or 1 wherein, if n is at least 3, in this formula II an amount of up to 1/3 of the radicals which are enclosed by the bracket can be replaced by radicals of the formula



R<sub>1</sub> represents a straight chain or branched alkyl group having 4 to 18 carbon atoms bound in the 6-, 4- or 2-position to the benzene nucleus,

R<sub>2</sub> represents hydrogen, a straight chain or branched alkyl group having 1 to 9 carbon atoms or a group of the formula



in which Y represents an alkyl group having 1 to 4 carbon atoms or the group  $-\text{C}_2\text{H}_4\text{OH}$ , A represents the anions  $\text{Cl}^{(-)}$ ,  $\text{Br}^{(-)}$ ,  $\text{I}^{(-)}$ ,  $\text{CH}_3\text{OSO}_3^{(-)}$ ,  $1/2-\text{SO}_4^{(2-)}$  in a quantity which is equivalent to the number of the positively charged sulfur atoms in the total molecule of the formula I.

2. An acid metal treating bath consisting essentially of hydrochloric acid and as corrosion inhibitor 0.05 to 2.0 percent by weight of a compound of the formula

| Product | Concentration, steel removal<br>(loss) in g./m. <sup>2</sup> |   |   |
|---------|--------------------------------------------------------------|---|---|
|         | a                                                            | b | c |

|     |       |       |       |
|-----|-------|-------|-------|
| 14. | 2,100 | 1,530 | 1,100 |
|-----|-------|-------|-------|

|     |       |       |       |
|-----|-------|-------|-------|
| 15. | 3,200 | 2,050 | 1,550 |
|-----|-------|-------|-------|

|     |       |       |       |
|-----|-------|-------|-------|
| 16. | 1,970 | 1,390 | 1,160 |
|-----|-------|-------|-------|



3. An acid metal treating bath consisting essentially of hydrochloric acid and as corrosion inhibitor 0.05 to 2.0 percent by weight of an equimolar mixture of the compounds of the formulae



4. An acid metal treating bath consisting essentially of hydrochloric acid and as corrosion inhibitor 0.05 to 2.0 percent by weight of a compound of the formula



5. An acid metal treating bath as claimed in claim 1, which additionally contains up to 15 percent by weight, referred to the sulfonium salt corrosion inhibitor, of an alkynol.

6. The acid metal treating bath as claimed in claim 1 wherein R<sub>2</sub> represents a group of the formula



wherein Y is an alkyl group of 1 to 4 carbon atoms.

7. The acid metal treating bath as claimed in claim 6  
wherein Y is -CH<sub>3</sub>.

8. An acid metal treating bath consisting essentially  
of hydro-chloric acid and as a corrosion inhibitor 0.05  
to 2.0 percent by weight of a compound of the general  
formula

10



\* \* \* \* \*

15

20

25

30

35

40

45

50

55

60

65